

## UNITED STATES PATENT OFFICE.

THEODOR LICHTENBERGER, OF HEILBRONN, AND KONRAD FLOR, OF BUCKEBURG, GERMANY.

## PROCESS FOR OBTAINING ALKALINE-EARTH-METAL SULPHIDES FROM ALKALINE-EARTH-METAL SULPHATES.

No Drawing. Application filed March 4, 1926, Serial No. 92,334, and in Germany May 8, 1925.

It has already been proposed to obtain sulphur from alkaline-earth-metal sulphates by dissolving the same in alkali-metal chloride in a molten condition. In this process, for the purpose of producing alkaline-earth-metal sulphide, carbon is employed either in the form of solid coal or in the form of reducing gases.

It has now been discovered that solid coal does not admit of being mixed well with the melt. The coal experiences owing to the degasification an upward drive and burns very quickly in the surface without being utilized for the reduction. The reduction is therefore only incomplete and requires a considerable expenditure of coal.

The process forming the subject-matter of the present invention is distinguished from the known process by the fact that the carbon is employed in the form of coke and that after the reduction a separation of the alkali-metal chloride from the alkaline-earth-metal sulphide is effected by sedimentation, whereupon the alkali-metal chloride is drawn off above, while the alkaline-earth-metal sulphide is converted in known manner by treatment with vapour or acid into alkaline-earth metal oxide or alkaline-earth-metal salt and hydrogen sulphide.

The coke admits of being mixed well with the melt and exerts a reducing action very quickly.

The invention is further based upon the discovery that the alkaline-earth-metal sulphides in the fused mass admit of being sharply separated from the alkali-metal chlorides by sedimentation. Consequently after the reduction only a clarification of the melt is necessary. The alkali-metal chloride may be drawn off above and employed afresh for dissolving alkaline-earth-metal sulphates. The alkaline-earth-metal sulphide obtained however is further treated, for the purpose of obtaining the hydrogen sulphide, in the manner mentioned above.

For the preparation of sodium sulphide and potassium sulphide from the corresponding sulphates by means of coal and common salt the use of coke has already been suggested. In the treatment of alkaline-earth-metal sulphates, however, coke has not hitherto been employed.

Magnesium chloride is preferably melted up with the melt which consists of alkali-

metal chloride and alkaline-earth-metal sulphide. By this means the conversion of the alkaline-earth-metal sulphides into alkaline-earth-metal chlorides is accelerated. The addition of the magnesium chloride may take place either before or after the reduction of the melt with coke.

Magnesium chloride has already been employed in the production of hydrogen sulphide in the wet way. This process however is costly and leads to the pollution of the waste waters.

The process may for example be carried out by introducing almost dehydrated magnesium chloride into the alkali metal chloride melt containing the reduced alkaline-earth-metal sulphates. Large quantities of hydrogen sulphide gas then escape with the elimination of magnesium oxide, while from the alkaline-earth-metal sulphides insoluble in the melt, alkaline-earth-metal chlorides are evolved which are readily soluble in the molten alkali-metal chlorides.

The evolution of hydrogen sulphide may be increased and accelerated if water vapour is passed into the melt.

In the manner described above a volatile melt free from alkaline-earth-metal sulphides is very quickly obtained which consists of alkali-metal chlorides and alkaline-earth-metal chlorides. In this melt the magnesium oxide is very quickly deposited, so that it can easily be removed.

If the melt of alkali-metal chlorides and alkaline-earth-metal chlorides freed from magnesia and still containing only the excess coke is utilized afresh for dissolving and reducing alkaline-earth-metal sulphates, the working process can firstly be made continuous and secondly the defects which are inherent in the wet process and which consist in the costly production of alkaline-earth-metal chlorides by evaporation or in the pollution of rivers by the waste waters can be eliminated in a technical simple manner.

Owing to the fact that the magnesia is always removed by sedimentation and the alkaline-earth-metal chloride that forms is returned to the cycle of operations, a pure alkaline-earth-metal chloride melt is finally obtained which only contains alkali-metal chlorides and the preparation of which is very simple and does not give rise to any worthless waste liquors to pollute the rivers.

Instead of sodium chloride it is possible to employ other alkali-metal or other alkaline-earth-metal salts or mixtures of such salts for melting up the alkaline-earth-metal sulphates. In this case salts must be selected which are fusible in an anhydrous condition and which do not exert any decomposing action when in a molten condition upon alkaline-earth-metal sulphates.

10 It has been discovered that the alkaline-earth-metal sulphates can easily be dissolved to a clear thinly liquid melt not only in molten sodium chloride but also in other molten alkali-metal or alkaline-earth-metal salts as 15 well as in molten mixtures thereof. Those alkali-metal or alkaline-earth-metal salts can be used which are particularly fusible in an anhydrous condition and which when in a molten condition exert no decomposing action 20 upon alkaline-earth-metal sulphates. Particularly suitable are the sulphates of the alkali metals as well as the fluorides of the alkali and alkaline-earth-metals either alone or mixed with other alkali-metal or alkaline-25 earth-metal salts.

If for example fluorspar is employed as a melting bath there are preferably mixed with it for the purpose of lowering the melting point alkali fluorides or alkaline-earth-30 metal chlorides. The same advantage is also obtained if an intimate mixture of alkali-metal or alkaline-earth-metal fluorides or alkaline-earth-metal chlorides is melted up with the alkaline-earth-metal sulphates 35 as its melting point lies far below the melting point of the individual components.

The fusible masses produced in this manner from alkaline-earth-metal sulphates with alkali-metal or alkaline earth salts or 40 with mixtures thereof are then further treated for obtaining the alkaline-earth-metal sulphate sulphur in the same manner as has been described above. Coke is stirred into the melt as a result of which the alkaline-45 earth-metal sulphate is reduced to alkaline-earth-metal sulphide and the latter, by blowing in steam or acid, is further decomposed into alkaline-earth-metal oxide or the corresponding alkaline-earth-metal salt and hydrogen sulphide which can then be further worked up in a known manner to sulphur or 50 sulphur compounds.

If alkali-metal or alkaline-earth-metal salts are employed which singly or mixed 55 in the melting bath split off acid when steam is blown in, after the reduction of the alkaline-earth-metal sulphates is terminated the alkaline-earth-metal sulphide obtained is decomposed by blowing in steam into alkaline-60 earth-metal salt and hydrogen sulphide as the acid that forms under the action of steam on the melting bath acts in a nascent condition upon the alkaline-earth-metal sulphide.

What we claim is:

65 1. Process for obtaining sulphur com-

pounds from alkaline-earth-metal sulphates, comprising dissolving the sulphate in molten sodium chloride, adding coke to obtain alkaline-earth-metal sulphide, separating the alkali-metal chloride from the alkaline-70 earth-metal sulphide by sedimentation and drawing off the alkali-metal chloride above.

2. Process for obtaining sulphur compounds from alkaline-earth-metal sulphates, comprising dissolving the sulphate in molten 75 sodium chloride, adding magnesium chloride and coke to the melt of alkali-metal chloride and alkaline-earth-metal sulphate and thereby obtaining alkaline-earth-metal sulphide and magnesium oxide, separating the alkali-80 metal chloride from the alkaline-earth-metal sulphide by sedimentation and drawing off the alkali-metal chloride above.

3. Process for obtaining sulphur compounds from alkaline-earth-metal sulphates, 85 comprising dissolving the sulphate in molten alkali-metal salts which are fusible without water and do not decompose alkaline-earth-metal sulphates when in a molten condition, adding coke to obtain alkaline-earth-metal sulphide, separating the alkali-metal salts from the alkaline-earth-metal sulphide by sedimentation and drawing off the alkaline-90 metal salts above.

4. Process for obtaining sulphur compounds from alkaline-earth-metal sulphates, comprising dissolving the sulphate in molten alkaline-earth-metal salts which are fusible without water and do not decompose alkaline-earth-metal sulphates when in a molten condition, adding coke to obtain alkaline-earth-metal sulphide, separating the alkaline-earth-metal salts from the alkaline-earth-metal sulphide by sedimentation and drawing off the alkaline-earth-metal salts above.

5. Process for obtaining sulphur compounds from alkaline-earth-metal sulphates, comprising dissolving the sulphate in a mixture of molten alkali-metal and alkaline-earth-metal salts which are fusible without water and do not decompose alkaline-earth-metal sulphates when in a molten condition, adding coke to obtain alkaline-earth-metal sulphide, separating the alkali-metal and alkaline-earth-metal salts from the alkaline-earth-metal sulphide by sedimentation and drawing off the alkaline-earth-metal salts above.

6. Process for obtaining sulphur compounds from alkaline-earth-metal sulphates, comprising dissolving the sulphate in molten alkali-metal salts which are fusible without water and do not decompose alkaline-earth-metal sulphates when in a molten condition, adding magnesium chloride and coke to the melt of alkali-metal salts and alkaline-earth-metal sulphate and thereby obtaining alkaline-earth-metal sulphide and magnesium oxide, separating the alkali-metal salts from

the alkaline-earth-metal sulphide by sedimentation and drawing off the alkali-metal salts above.

7. Process for obtaining sulphur compounds from alkaline-earth-metal sulphates, comprising dissolving the sulphate in molten alkaline-earth-metal salts which are fusible without water and do not decompose alkaline-earth-metal sulphates when in a molten condition, adding magnesium chloride and coke to the melt of alkaline-earth-metal salts and alkaline-earth-metal sulphate and thereby obtaining alkaline-earth-metal sulphide and magnesium oxide, separating the alkaline-earth-metal salts from the alkaline-earth-metal sulphide by sedimentation and drawing off the alkaline-earth-metal salts above.
8. Process for obtaining sulphur compounds from alkaline-earth-metal sulphates,

comprising dissolving the sulphate in a mixture of molten alkali-metal and alkaline-earth-metal salts which are fusible without water and do not decompose alkaline-earth-metal sulphates when in a molten condition, 25 adding magnesium chloride and coke to the melt of alkali-metal salts and alkaline-earth-metal salts and alkaline-earth-metal sulphate and thereby obtaining alkaline-earth-metal sulphide and magnesium oxide, separating the alkali-metal and alkaline-earth-metal salts from the alkaline-earth-metal sulphide by sedimentation and drawing off the alkali-metal and alkaline-earth-metal salts above. 30 35

In testimony whereof we have signed our names to this specification.

THEODOR LICHTENBERGER.  
KONRAD FLOR.